# EUROPEAN PATENT SPECIFICATION

(11) **EP 1 045 040 B1**
(45) Date of publication and mention of the grant of the patent: **12.01.2005**
(21) Application number: 99500058.5
(22) Date of filing: 15.04.1999
(51) Int. Cl.: C22C 1/02, B22F 1/00, C22B 9/10

(54) **Additive for adding one or more metals into aluminium alloys**
Zusatzmittel zur Zuführung von Metallen in Aluminiumlegierungen
Additif pour ajouter des métaux aux alliages d'aluminium

(43) Date of publication of application: 18.10.2000
(73) Proprietor: Bostlan, S.A., 48100 Mungia (Bizkaia) (ES)
(72) Inventor: Diaz Maruri, Francisco, 48509 Abanto (Bizkaia) (ES); Arco González, Aitor, 48006 Bilbao (ES); Posada Fernández, Tomás, 48100 Mungia (Bizkaia) (ES); Elustondo Amorrortu, Javier, 48990 Algorta-Getxo (Bizkaia) (ES)
(74) Representative: Carpintero Lopez, Francisco

(56) References cited:
- GB-A- 2 112 020
- GB-A- 2 117 411
- US-A- 4 581 069
- US-A- 4 820 483
- US-A- 5 342 573
- "Metals Handbook, 9th Edition, Vol.7" 1984 , AMERICAN SOCIETY FOR METALS , OHIO, USA XP002119041 * page 190 - page 193 *
- R. M. GERMAN: "Powder Injection Molding" 1990 , METAL POWER INDUSTRIES FEDERATION , NEW JERSEY USA XP002119042 * page 99 - page 124 * * page 114, paragraph 3 * * page 104, paragraph 2; table 4.2 *

## Description

This invention relates to an additive for adding one or more metals in aluminium alloys, as well as the way the metals are added into a melting aluminium.

The use of fluxes such as fluorides, chlorides and carbonates in the alloy tablets in this industrial applications presents some drawbacks related to the significant environmetal problems they imply, and to the presence of inclusions in the obtained alloys. Thus, new fluxes of different characteristics are necessary in order to improve the features of the metals dissolution in relation to those given by the tablets with no flux currently used.

References US-A-4.880.462, US-A-4.564.393 and UK-A-2.112.020 present an additive for this application, but the flux is of hazardous nature and makes it possible to form inclusions in the aluminium.

Reference GB-A-2.267.455 proposes the application of waxes in a different field: the powder metallurgy.

US 4581069 describes the formation of a master alloy by compacting non-spherical particles and using an organic binder, which is burnt off as the master alloy briquette is introduced into the molten metal mass.

When inserted into the melting aluminium, the additive of this invention yields important improvements, collected in the following aims:
* an aim of the invention is an additive for increasing the dissolution velocity of the added metals,
* another aim of the invention is an additive for increasing the recovery of the added metals,
* another aim of the invention is an additive for producing a stirring effect in the melting aluminium, in order to increase the homogeneous distribution of the metal throughout the whole alloy,
* another aim of the invention is to provide a reduction of the impurities in the melting aluminium, since the produced gases promote their buoyancy,
* finally, another aim of the invention is to reduce the amount of added metal accumulated in the bottom of the furnace.

In order to carry out this aims, the invention claims an additive for adding one or more metals in the aluminium alloys. This additive contains:
(a) an agglutinating powder, for example, commercial powder aluminium, magnesium or an alloy or mixture of both of them,
(b) a powder of one or more metals or alloys comprising that or those to be added, for example, manganese, chromium, tungsten, molybdenum, titanium, vanadium, iron, cobalt, copper, niobium, nickel, tantalum, zirconium, hafnium, silver, lead, zinc, and,
(c) a wax-type organic compound.

The weight proportions in the final mixture are:
(a) from >0% to 49.9%,
(b) from 50% to 95%,
(c) from 0.1% to 5%.

Any aluminium alloy containing acceptable amounts of materials with a unfavourable effect in the final aluminium alloy can be used as the component (a), but it is better to use as pure as possible aluminium, so commercially pure aluminium is recommended for component (a).

The best weight proportion (A) for the aluminium component should satisfy A≤49.9%. A proportion about 20% is preferred.

These additives are used in order to add metals of higher melting point than that of the aluminium into the melting aluminium, for example, manganese, chromium, tungsten, molybdenum, titanium, vanadium, iron, cobalt, copper, niobium, nickel, tantalum, zirconium, hafnium, and silver, and, especially, manganese, chromium, titanium, iron and copper. The metallic component added is usually formed by one or more commercially pure metals, but it can be one or more alloys of such metals, taking into account that this alloy or alloys should not lead to unacceptable amounts of undesirable compounds into the melting aluminium.

If different metals have to be added into the melting aluminium at the same time, one or more metals can be added using an additive according to this invention, and other procedures can be used for inserting the rest of the metals. The different metals to be added by means of an additive according to this invention should be present in the additive as:
(1) a mixture of the powders of the metals,
(2) a powder of an alloy of the metals,
(3) a mixture of the powders of, at least one alloy and at least one metal.

The weight proportion (B) for the component (b) should satisfy the condition: 50%<B<95%. This condition makes the metallic component (b) to reach reasonable concentrations in the additive whereas high dissolution rates and recoveries of the added metal are obtained. A proportion between 75% and 80% is preferred for B.

The flux must be a wax. Any kind of wax can be used, but it should rather be a non-polar one. More specifically, a wax with no impurities being harmful for the melting aluminium, for example, paraffin or polyethylene waxes, should be used.

We have found the best results for a weight proportion C of the component (c) satisfying the condition 0.1%≤C≤5%, preferably in the range 0.3%≤C≤1%. C values less than 0.3% produce clearly minor benefits than the maximum, and C values higher than 5% are not desirable, since smokes from the combustion of the wax are produced, dross appears on the surface of the melting aluminium, and hydrogen and carbon are inserted into the aluminium.

According to this invention, a highly recommended additive includes commercially pure aluminium for the component (a), with A values about 19%, B values about 80% and C values about 1%. The more desirable products for the additives described in this paragraph are commercially pure chromium, commercially pure manganese, commercially pure iron or commercially pure titanium.

The particle sizes of the aluminium component and that of the added metal component should preferably be less than 1 mm. The size of the wax particles should preferably be less than 0,5 mm.

Components are easier to insert and maintain into the melting aluminium when they are added by means of a body formed by compression of its components. Such bodies should be formed by compressing powdered mixtures of components (a), (b) and (c) using, for example, a press or an horizontal hydraulic machine for produce tablets.

The melting aluminium bath to be alloyed can be commercially pure, which is usually known as primary aluminium, or an alloy from a secondary melting.

In order to provide a better understanding of the invention some examples and claims are enclosed.

### EXAMPLE 1

Three mixtures with the following weight proportions of the components were prepared:
(a) 80% of electrolytic manganese powder with 0,55% oxidation level.
(b) 0%, 0,5% and 1% of paraffin wax.
(c) 20%, 19,5 and 19% of aluminium powder, respectively.

The mixtures were pressed in a vertical hydraulic press to give them a tablet shape, with about 90 mm diameter and 25 mm height. The tablets contained exactly 500 g of manganese and the total weight was about 625 g. The tablets were named ALMEN 0,5-80M.

Three independent experiments were performed in a 50 Kg capacity electric melting furnace. The initially added charge was 50 Kg of 1070 aluminium alloy. After melting of the aluminium, temperature was adjusted to 720°C. The dross was removed from the surface and the blank sample was taken. The referred tablets were added and it was observed that the bigger the proportion of wax in the added sample, the higher stirring effect obtained into the melting aluminium. The aluminium bath was adequately stirred and control samples were taken in order to know the dissolution process of the manganese into the alminium as a function of time. Figure 1 shows the percentages of Mn recovered versus time for different contents of wax.

It can be seen in the plots that high levels of wax in the tablet imply a faster dissolution process and a higher final manganese recovery.

The initial and final levels of manganese in the melting aluminium, as well as the temperatures registered during the three different processes are completely comparable.

### EXAMPLE 2

Two mixtures with the following weight proportions of the components were prepared:
(a) 75% of electrolytic manganese powder.
(b) 0%, and 0,5% of paraffin wax.
(c) 25% and 24,5% of aluminium powder, respectively.

The mixtures were pressed in an horizontal hydraulic press to give them a briquette shape, with about 40,5 mm diameter and 40 mm height. The total weight of the briquettes is 200 g and they contain 150 g of manganese. The briquettes were named ALMEN 275M.

Two independent experiments were performed in a 10 metric tons oxyfuel furnace. About 9 metric tons of 1070 aluminium alloy were added to the furnace in order to obtain a commercial 3003 aluminium. After melting of the aluminium in the melting furnace, aluminium was transferred to a holding furnace, where temperature was adjusted to about 720°C for both experiments. At that time, surface dross was removed and a blank sample was taken. 120 briquettes were added, and similar phenomena to those in the Example 1 were observed. Aluminium was adequately stirred, and control samples were taken in order to know the dissolution process of the manganese briquettes into the aluminium as a function of time. Figure 2 shows the percentages of Mn recovered versus time for different contents of wax.

It can be seen in the plots that high levels of wax in the tablet imply a faster dissolution process and a higher final manganese recovery.

## Claims

1. An additive for adding one or more metals in aluminium alloys which comprises :
- (a) an agglutinating powder comprising aluminium, magnesium or a mixture or alloy thereof
- (b) a powder of one or more metals or alloys comprising that or those to be added, for example, manganese, chromium, tungsteno, molybdenum, titanium, vanadium, iron, cobalt, copper, niobium, nickel, tantalum, zirconium, hafnium, silver, lead, zinc,
- (c) a wax-type organic compound, following the next weight proportions in the final mixture: from >0% to 49.9% for component (a), from 50% to 95% for component (b) and from 0,1% to 5% for component (c).

2. An additive for the introduction of one or more metals into the aluminium alloys, according to the 1st claim **characterized in that** the component (a) is a powder of commercial aluminium.

3. An additive for the introduction of one or more metals into the aluminium alloys, according to the 1st claim, **characterized in that** the component (a) is a powder of aluminium and magnesium.

4. An additive for the introduction of one or more metals into the aluminium alloys, according to the 1st claim, **characterized in that** the component (a) is a powder of commercial magnesium.

## Patentansprüche

1. Ein Zusatz zum Hinzufügen eines oder mehrerer Metalle zu Aluminiumlegierungen, der Folgendes umfasst:
- (a) ein Klebepulver, das Aluminium, Magnesium oder eine Mischung oder eine Legierung enthält.
- (b) ein Pulver aus einem oder mehreren Metallen oder Legierungen, die diese oder die hinzuzufügenden enthalten, zum Beispiel Mangan, Chrom, Tungsten, Molybdän, Titan, Vanadium, Eisen, Kobalt, Kupfer, Niob, Nickel, Tantal, Zirkon, Hafnium, Silber, Blei, Zink
- (c) eine wachsähnliche organische Zusammensetzung gemäss den folgenden Gewichtsverhältnissen in der Endmischung: >0% bis 49,9% der Komponente (a), zwischen 50% und 95% der Componente (b) und zwischen 0,1% und 5% für die Komompente (c).

2. Ein Zusatz zum Hinzufügen eines oder mehrerer Metalle zu den Aluminiumlegierungen, gemäss Anspruch 1, **dadurch gekennzeichnet, dass** die Komponente (a) das Pulver eines Handelsaluminiums ist.

3. Ein Zusatz zum Hinzufügen eines oder mehrerer Metalle zu den Aluminiumlegierungen, gemäss Anspruch 1, **dadurch gekennzeichnet, dass** die Komponente (a) das Pulver von Aluminium und Magnesium ist.

4. Ein Zusatz zum Hinzufügen eines oder mehrerer Metalle zu den Aluminiumlegierungen, gemäss Anspruch 1, **dadurch gekennzeichnet, dass** die Komponente (a) das Pulver eines Handelsmagnesiums ist.

## Revendications

1. Un additif pour ajouter un ou plusieurs métaux dans des alliages d'aluminium qui comprend :
- (a) une poudre agglutinante comprenant de l'aluminium, du magnésium ou un mélange ou un alliage;
- (b) une poudre d'un ou plusieurs métaux ou alliages comprenant celui ou ceux à ajouter, par exemple, le manganèse, le chrome, le tungstène, le molybdène, le titane, le vanadium, le fer, le cobalt, le cuivre, le niobium, le nickel, le tantale, le zirconium, l'hafnium, l'argent, le plomb, le zinc,
- (c) un composé organique de type cire, suivant les proportions de poids suivantes dans le mélange final: de >0% à 49,9% pour le composant (a), de 50% à 95% pour le composant (b) et de 0,1% à 5% pour le composant (c).

2. Un additif pour l'introduction d'un ou plusieurs métaux dans les alliages d'aluminium, selon la revendication 1, **caractérisé en ce que** le composant (a) est une poudre d'aluminium commercial.

3. Un additif pour l'introduction d'un ou plusieurs métaux dans les alliages d'aluminium, selon la revendication 1, **caractérisé en ce que** le composant (a) est une poudre d'aluminium et de magnésium.

4. Un additif pour l'introduction d'un ou plusieurs métaux dans les alliages d'aluminium, selon la revendication 1, **caractérisé en ce que** le composant (a) est une poudre de magnésium commercial.
